

# UNITED STATES PATENT OFFICE.

ROBERT C. TOTTEN, OF PITTSBURG, PENNSYLVANIA.

## COMPOSITION OF METAL.

No. 872,483.

Specification of Letters Patent.

Patented Dec. 3, 1907.

Application filed December 22, 1906. Serial No. 349,169.

*To all whom it may concern:*

Be it known that I, ROBERT C. TOTTEN, a resident of Pittsburg, in the county of Allegheny and State of Pennsylvania, have invented a new and useful Improvement in Composition of Metal; and I do hereby declare the following to be a full, clear, and exact description thereof.

My invention relates to a composition of chilling cast iron, and to the manufacture of the same and the articles produced therefrom, its object being to provide from what are known as coke or coal irons, that is, pig metal smelted with coke or anthracite coal, what is known as a "chilling" cast iron, that is, a metal suitable for the manufacture of castings of great strength and fineness of grain, such as chilled castings, which have heretofore been made principally from what is known as charcoal iron, the same character of iron being also adapted for the making of malleable castings and for some other uses requiring special strength. Charcoal pig metal has generally been considered a necessity for the manufacture of such chilled castings, the generally understood reason for this being that it is the only pig metal that contains what is termed "combined carbon" in sufficient quantity to impart to the iron containing it the peculiarity of making a chilled surface when cast against a metal chill. One theory in regard to this "combined carbon" is that the carbon is chemically united or combined with the iron as distinguished from being present in graphitic form. While the demand for this charcoal pig iron has been constantly increasing the production of the same has apparently reached its limit, largely on account of the cost of the charcoal necessary for smelting the same.

By my invention I am able to produce from pig iron made by the coke or coal process a chilling cast metal having practically the same properties as found in the charcoal pig iron and thus to utilize a cheaper pig iron for the purpose and one of which there is abundant supply.

My invention consists, generally stated, in a new composition of "chilling" cast metal, consisting of coke or coal iron and a chromium compound containing combined iron and carbon, such as ferro chrome; the ferro-chrome containing a large proportion of such combined iron and carbon and providing in the chilling cast iron so formed

a sufficient proportion of combined carbon to give to that metal the peculiar qualities ordinarily found in charcoal iron as above referred to, while the chrome present adds to the hardness without reducing the strength of the casting so produced. In the manufacture of this chilling cast iron I melt the coke or coal iron in any suitable way, preferably in an air furnace, and I also prefer to melt the ferro-chrome. I may either melt the iron in one furnace, and melt the ferro-chrome in another furnace or crucible, and add it to the iron, regulating it as found desirable to produce the proper depth of chill which may be tested while the metal is still molten; or I may add the ferro chrome in solid state to the molten iron in the furnace, or I may add the molten or solid ferro-chrome in the ladle which receives the iron from the melting furnace; in this way uniting the two metals or alloys in any suitable or effective way.

The ordinary coke or coal pig iron contains a large amount of graphitic carbon and a small proportion, sometimes only a trace, of combined carbon. Ferro-chrome contains a large proportion of combined carbon ranging as high as ten (10) to twelve (12) per cent. These metals I mix in suitable proportions in order to obtain the requisite amount of combined carbon in the resultant casting iron, it being desired that this proportion shall be as much as one quarter of one per cent. ( $\frac{1}{4}$  of 1%) of combined carbon for strong, fine grained castings, and as much as one (1) per cent. or over for chilled rolls, car wheels, etc. For this purpose I can vary the amount of ferro-chrome in any desired proportion, being melted together or melted separately and then mixed in any suitable way, to produce a casting with suitable strength and fineness of grain for a chilled roll, car wheel and the like, the chill usually being from one half ( $\frac{1}{2}$ ) inch to two (2) inches in depth. As an illustration—using coal or coke iron with, say, one quarter of one per cent. ( $\frac{1}{4}$  of 1%) combined carbon, and ferro-chrome containing ten (10) per cent. combined carbon, a mixture would be produced by using twenty to twenty-five per cent (20 to 25%) of such ferro-chrome containing two (2) to two and one half ( $2\frac{1}{2}$ ) per cent. combined carbon, producing a high chilling iron. Or by using the same grade of pig iron and using twenty (20) to twenty-five (25) per cent. of ferro-chrome containing six (6) per cent. combined

carbon, a chilling iron would be produced of moderate chilling properties. I have found that in this way I am enabled to produce a casting iron of fine grain and great strength 5 adapted to produce castings of the character referred to and especially chilled rolls, car wheels, etc., with a hard wearing surface and the necessary strength back of the chilled surface in the body of the roll or car wheel.

10 It may also be employed to advantage for malleable castings, cylinders and the like requiring special strength.

As the supply of charcoal iron is limited, and the supply of ordinary coke or coal iron 15 is practically unlimited I am thus enabled to produce a cheap and suitable substitute for the ordinary charcoal iron, and one which produces a harder and more durable wearing surface.

20 What I claim is:

1. A new composition of chilling cast iron, consisting of coke or coal iron and a chro-

mium compound containing combined iron and carbon.

2. A new composition of chilling cast iron, 25 consisting of coke or coal iron and ferro-chrome.

3. A new composition of chilling cast iron, consisting of coke or coal iron and a chromium compound containing combined iron 30 and carbon, the composition containing at least one-fourth ( $\frac{1}{4}$ ) of one (1) per cent. of combined carbon.

4. A new composition of chilling cast iron, consisting of coke or coal iron and ferro 35 chrome containing at least one fourth ( $\frac{1}{4}$ ) of one (1) per cent. of combined carbon.

In testimony whereof, I the said ROBERT C. TOTTEN have hereunto set my hand.

ROBERT C. TOTTEN.

Witnesses:

M. V. KIEHL,  
H. M. CORWIN.